

## UNITED STATES PATENT OFFICE.

SRINIVAS RAM WAGEL, OF NEW YORK, N. Y., ASSIGNOR TO THE LEHIGH COAL AND NAVIGATION COMPANY, A CORPORATION OF PENNSYLVANIA,

## PROCESS FOR BRIQUETTING BITUMINOUS COAL.

No Drawing. Application filed June 16, 1924, Serial No. 720,451. Renewed July 31, 1926.

This invention relates to a process for making briquettes of bituminous coal dust, or slack, whereby a hard and substantially smokeless fuel results; and it comprises 5 more specifically a process wherein soft coal dust is mixed by steam with a sulphite binder such as is disclosed in my copending application, Serial Number 708,571, and clay; and subsequently briquetted before finally passing the unfinished product 10 through a series of furnaces, the passage through each furnace serving to alternately heat and cool the briquette, and the successive heatings in each furnace being at increasing 15 temperatures, as and for the purpose to be hereinafter more specifically described and claimed.

Attempts have been made in the past to utilize bituminous coal dust as a fuel, but 20 such attempts have not met with any material degree of success. The use of such slack as fuel is most generally obtained by mixing it with anthracite coal, but the burning quality of the hard coal is not improved 25 by such mixing, and the quantity which can be mixed without objectionable effects is decidedly limited.

Briquettes have also been made of bituminous coal, usually with an asphalt binder, 30 but such briquettes have been found to deform under pressure and heat, and are further objectionable in that they emit a large amount of smoke in burning.

It is an object of the present invention to 35 make a briquette of soft coal dust, which is capable of withstanding heat and pressure without deformation, and which is practically smokeless in burning.

A further object is to so harden briquettes 40 made of soft coal that they are substantially waterproof, capable of withstanding crushing stresses, and not subject to deformation and stickiness within all the ordinary ranges of temperature.

45 A still further object is to make a hard and practically smokeless fuel from bituminous coal.

These objects, together with others which 50 will be apparent as the description proceeds, are accomplished by the following process:—

About ninety parts of soft coal dust, or slack, is mixed with approximately five parts of clay, and five and one-half parts of a sulphite binder such as is described in 55 my copending application, Serial Number

708,571, filed April 23, 1924. Such sulphite binder is composed of a mixture of sulphite liquor, clay and asphalt in the approximate proportions of forty to thirteen to twenty-seven, respectively. The mixing of slack 60 with the sulphite binder and clay is accomplished by steam.

The mass resulting from such mixing is then passed through a machine of any conventional type for moulding it into a plurality of briquettes.

After being formed into briquettes the unfinished product is passed along a series of superposed endless conveyor belts, each of which passes through a furnace such as is 70 shown in my copending application, Serial Number 709,181. The furnace is formed with a plurality of vertically aligned tunnels, each of which is open at both ends, and through each of which an endless conveyor passes and extends for four or five feet beyond. In the present process I prefer to use a furnace having five tunnels, and to so time the speed of the conveyors therethrough, that the passage of the briquettes 80 through each tunnel consumes about four minutes.

It has also been found necessary to use a battery of such furnaces, preferably twelve to sixteen in number, so that the heating 85 process is carried to an extent whereby, when the finished product finally emerges, it is in reality a coal brick due to the baking of the clay content therein.

The operation of the furnaces is as follows: 90

When the unfinished briquette leaves the moulding machine it is dropped onto a conveyor and slowly passed through the uppermost of the vertical tier of tunnels in the first furnace. This tunnel, being uppermost, is less hot than those beneath it, and consequently the briquette is not raised to a very high temperature during this step of the hardening process. After leaving the first tunnel it passes, on the same conveyor, 100 to a point four or five feet beyond where it is dropped onto the next lower conveyor, and passed back through the furnace at the next lower level, being heated to a higher temperature than previously. This 105 action continues, each heating being higher than the previous one, and the successive heatings being alternated by a cooling outside of the furnace, during which the temperature of the briquette drops 200° to 300° 110

Fahrenheit. Each heating expands the briquette, and each subsequent cooling contracts it, so that as it passes through the furnace, the constituent materials are firmly knit together.

After passing through the lowermost of the tunnels in the first furnace, the briquette is next passed to the uppermost tunnel of the second furnace where its travel is the same as previously. This process is carried on until the briquette has been passed through a battery of from twelve to sixteen furnaces as has already been pointed out.

During the heating of the briquette in the furnaces, it is not only hardened, but a large amount of the volatile matter contained in the coal and binder is driven therefrom, so that the resulting product will burn with a minimum amount of smoke.

The briquette produced by the process above set forth is a coal brick, the strength of which is seven or eight times that of bituminous coal, and which possesses all of the desirable qualities of such fuel, while at the same time, those which are objectionable are eliminated.

Having described my invention, what I claim is:—

1. In the manufacture of coal briquettes, the process which comprises mixing bituminous coal with clay and a binder of sulphite liquor, clay and asphalt; and in passing the mixture through regions of increasing temperature, with alternate cooling thereof.

2. In the manufacture of coal briquettes, the process which comprises mixing bituminous coal with clay and a binder composed of sulphite liquor, clay, and asphalt, by means of steam; in alternately heating and cooling such mixture, the successive heatings being at increasingly higher temperatures.

3. In the manufacture of coal briquettes, the process which consists in mixing through the medium of steam, bituminous coal, clay, and a binder composed of sulphite liquor, clay, and asphalt; in moulding such mixture into briquettes; in passing the bri-

quettes so formed through regions of increasing temperature; in cooling the briquettes between each successive heating; and in finally repeating the heating and cooling process.

4. In the manufacture of coal briquettes, the process which comprises mixing bituminous coal with a binder of sulphite liquor, clay and asphalt, briquetting the mixture and baking the same sufficiently to drive out a substantial amount of volatile matter and harden the briquettes.

5. In the manufacture of coal briquettes, the process which comprises mixing bituminous coal with a binder of sulphite liquor, clay and asphalt, briquetting the mixture and subjecting the briquettes thus formed to alternate heating and cooling.

6. In the manufacture of coal briquettes, the process which comprises mixing bituminous coal with clay and a binder of sulphite liquor, clay and asphalt, forming the mixture into briquettes and baking the briquettes sufficiently to drive out a substantial amount of volatile matter and harden the briquettes.

7. A coal briquet comprising bituminous coal and a binder of sulphite liquor, clay and asphalt which has been baked sufficiently to drive out a substantial amount of volatile matter and harden the briquettes.

8. A coal briquet comprising bituminous coal, clay and a binder of sulphite liquor, asphalt and clay which has been baked sufficiently to drive out a substantial amount of volatile matter and harden the briquettes.

9. A coal briquette comprising bituminous coal and a binder of sulphite liquor, asphalt and clay which has been subjected to alternate heating and cooling steps to expand and contract the same.

10. A coal briquette comprising bituminous coal, clay and a binder of sulphite liquor, clay and asphalt which has been subjected to alternate heating and cooling steps to expand and contract the same.

In testimony whereof I affix my signature.

SRINIVAS RAM WAGEL.